

1

2,942,930

## ALUM TANNAGE

Fred P. Luvisi, Elkins Park, William F. Happich, Jenkintown, Mary V. Hannigan, Lafayette Hill, and Clarence W. Beebe, Roslyn, Pa., assignors to the United States of America as represented by the Secretary of Agriculture

No Drawing. Filed Nov. 7, 1958, Ser. No. 772,639

2 Claims. (Cl. 8—94.29)

(Granted under Title 35, U.S. Code (1952), sec. 266)

A non-exclusive, irrevocable, royalty-free license in the invention herein described, throughout the world for all purposes of the United States Government with power to grant sublicenses for such purposes, is hereby granted to the Government of the United States of America.

This application is a continuation-in-part of our pending application entitled "Alum Tannage," filed October 30, 1956, Serial No. 619,363, now abandoned.

This invention relates to a new method of tanning skins.

The tannage of leather by the use of aluminum salts is an old, well-known process. However, the tannage is commonly known to be unstable, yielding leathers of poor heat and water resistance. It is quite reversible; the loosely combined alum is poorly fixed in the leather, hydrolyses readily, and is easily removed by washing with water.

An object of this invention is to make a more stable and irreversible alum tannage.

Another object of the present invention is to produce an alum-tanned leather which may be fat-liquored satisfactorily in aqueous fat-liquoring systems similar to those employed in the leather-making trade.

A further object is to provide an alum-tanned leather which may be retanned successfully with vegetable tannin.

In general, according to the invention, the skins are impregnated with a solution of a water soluble aluminum salt until the skins are tanned in a usual manner. The tanned skins are then subjected to the action of a homopolymer of acrylic acid, of sodium polyacrylate, or of ammonium polyacrylate to fix the aluminum salt in the tanned skins. The skins are then fat-liquored in an aqueous fat-liquoring treatment similar to that employed in the leather making trade. A white leather is produced.

Although the initial appearance of skins which have been tanned by applying the same reagents in reverse order, or by simultaneous application of the reagents, indicates a tannage to give a somewhat comparable white leather, quite unexpectedly only the combination of the present invention, that is, impregnating with a solution of a water soluble aluminum salt followed by subjecting the tanned skins to the action of a homopolymer of acrylic acid, of sodium polyacrylate, or of ammonium polyacrylate, gives a leather which upon fat-liquoring in a typical aqueous fat-liquoring system results in a satisfactory product. The finished leather resulting from the present invention is especially suitable for upholstery, gloves, or other uses where a soft, flexible leather is essential to high quality products.

The first part of the process, commonly referred to as an alum tannage, comprises impregnating the skins with a solution of a water soluble aluminum salt. Commercially available basic aluminum acetate, such as  $\text{Al}(\text{OH})_2(\text{OOCCH}_3)_3 \cdot \frac{1}{2} \text{H}_2\text{BO}_3$ , may be used. Alum or aluminum sulfate, adjusted to the desired degree of

2

basicity, which may require the addition of a "masking" agent such as sodium acetate, sodium citrate or sodium tartrate in the proportion of one mole of "masking" agent to one mole of aluminum sulfate, have also been used. The pH of the solution may be varied from 4.2 to 6.5 and the time of treatment from 4 hours to 48 hours, depending upon the type of skins used and the kind of leather desired. The amount of aluminum in the finished leather, determined as  $\text{Al}_2\text{O}_3$  and usually 2.5 to 6%, may be controlled by varying the tanning conditions. The operation is conducted in a drum, paddle, or by other suitable methods.

The second part of the inventive process comprises treating the skins, after a short wash in water, with a solution of the homopolymer of acrylic acid, or with sodium polyacrylate or ammonium polyacrylate, containing approximately 2% polymer based on the wet drained weight of the skins, for 8 to 24 hours. Commercially available polymer preparations, representing low molecular weight polymer and high molecular weight polymer, were employed in operating the process. At the time the solution of polymer is being applied the pH should preferably be in the range of about 4.5 to 5.0.

After tanning the standard procedure is to fat-liquor the tanned skins. A dyeing step may precede the fat-liquoring in commercial practice. Fat-liquoring comprises drumming the skins in an aqueous oil emulsion. Oils conventionally employed are raw and sulfated neatsfoot oil, raw and sulfated sperm oil, combinations of these oils with a vegetable oil such as coconut oil, and rice bran oil. Several proprietary oils containing mixtures of the typical oils used in the trade were employed to satisfactorily fat-liquor skins tanned by the process of the present invention. In all instances the area shrinkage of the skin and loss of aluminum salt during fat-liquoring were negligible and a strong, soft, flexible leather was obtained. In contrast, comparative skins tanned by applying the polymer to the skin prior to tanning with the aluminum salt, or by applying the polymer and the aluminum salt in the same solution, did not fat-liquor satisfactorily, resulting in hard leathers, oily on the surface, which had shrunk excessively, sometimes as much as one-third of the original area.

Some typical illustrations of the application of the present invention are presented in the following examples:

## Example I

A piece of pickled calfskin was drummed intermittently in a solution of a water soluble basic aluminum acetate containing 4%  $\text{Al}_2\text{O}_3$  based on the wet drained weight of skin (33 grams) and 10% (w/v.)  $\text{NaCl}$ . Float ratio was 3 to 4 times wet weight skin. After 21 hours the pH was 4.5. This was adjusted to pH 6.0–6.5 with borax and the drumming continued 3 hours. The skin was removed, washed 5 minutes in lukewarm water, drained, and drummed intermittently in a solution of high molecular weight homopolymer of acrylic acid containing 2% polymer based on wet drained weight of skin and 10% (w/v.)  $\text{NaCl}$  for a period of 24 hours. Float ratio was about 7 times weight of wet skin. The pH of the polymer solution was 3.10 at the start and 4.50 after 24 hours. The leather was washed 10 minutes in lukewarm water, drained and cut in half. One half was fat-liquored in an aqueous oil emulsion system similar to that used in the trade for mineral tanned skins, drumming for one and one-half hours at 120° F., removed, and tacked out to dry. The other half was drummed intermittently in a 42° Bk sulfited quebracho solution for 20 hours, washed 2 minutes with water, fat-liquored as described, and tacked out to dry. The alum-polyacrylic acid tannage produced a uniformly white, full, pliable,

well-tanned leather with an even, close grain, having a shrinkage temperature of 87° C. Retannage of this leather with sulfited quebracho produced a uniformly tanned, soft, pliable leather of good color and having a shrinkage temperature of 103° C.

*Example II*

A piece of pickled calfskin was drummed intermittently in a solution of a water soluble basic aluminum acetate containing 4%  $\text{Al}_2\text{O}_3$  based on the wet drain weight (51 grams) and 10% (w/v.)  $\text{NaCl}$ . Float ratio was 3 to 4 times wet weight. After 21 hours the pH was 4.5. This was adjusted to pH 6.0-6.5 with borax and the drumming continued 3 hours. The skin was then removed, washed 5 to 10 minutes in lukewarm water, drained and drummed intermittently in a solution of high molecular weight sodium polyacrylate containing 2% polymer on wet drained weight skin and 10% (w/v.)  $\text{NaCl}$  for a period of 24 hours. Float ratio was 5 times wet weight. The pH of the sodium polyacrylate solution was 7.97 at the start and was adjusted with lactic acid so that at the end of the 24-hour period the pH was 4.8. The leather was washed 10 minutes in lukewarm water, drained and cut in half. One-half was fat liquored with a commercial fat-liquoring oil in the conventional aqueous system and tacked out to dry. The other half was drummed intermittently in a 42° Bk. sulfited quebracho solution for 20 hours, rinsed 2 minutes with water, fat-liquored with a nonionic oil and tacked out to dry. The alum-sodium polyacrylate tannage produced a white leather that was quite full, pliable and well tanned with a shrinkage temperature of 91° C. Retannage of this leather with sulfited quebracho produced a plump, well-tanned leather of uniform color with a shrinkage temperature of 116° C.

*Example III*

A piece of pickled calfskin was drummed intermittently in a solution of a water soluble basic aluminum acetate containing 4%  $\text{Al}_2\text{O}_3$  based on the wet drained weight (51 grams) and 10% (w/v.)  $\text{NaCl}$ . Float ratio was 3 to 4 times wet weight. After 22 hours the pH was 4.6. This was adjusted to pH 6.6 with borax and the drumming continued 4 hours. The skin was then removed, washed 5 minutes in lukewarm water, drained and drummed intermittently in a solution of low molecular weight polyacrylic acid containing 2% polymer on wet drained weight of skin and 10% (w/v.)  $\text{NaCl}$  for a period of 24 hours. Float ratio was 5 times wet weight. The pH of the polyacrylic acid solution was 2.80 at the start and 4.79 after 24 hours. The leather was washed 10 minutes in lukewarm water, drained and cut in half. One-half was fat-liquored in an aqueous system containing a proprietary nonionic oil and tacked out to dry. The other half was drummed intermittently in a 46.5° Bk. sulfited quebracho solution for 20 hours, rinsed 2 minutes with water, fat-liquored with a nonionic oil and tacked out to dry. The alum-polyacrylic acid tannage produced a white, full, soft, pliable leather with a shrinkage temperature of 87° C. Retannage of this leather with sulfited quebracho produced a soft, plump, fully tanned leather of even color and with a shrinkage temperature of 112° C.

*Example IV*

A piece of pickled calfskin was drummed intermittently in a solution of a water soluble basic aluminum acetate containing 4%  $\text{Al}_2\text{O}_3$  based on the wet drained weight (49 grams) and 10% (w/v.)  $\text{NaCl}$ . Float ratio was 3 to 4 times wet weight. After 22 hours the pH was 4.6. This was adjusted to pH 6.6 with borax and the drumming continued 4 hours. The skin was then removed, washed 5 minutes in lukewarm water, drained and drummed intermittently in a solution of low molecular weight sodium polyacrylate containing 2% polymer on wet drained weight of skin and 10% (w/v.)  $\text{NaCl}$  for a period of

24 hours. Float ratio was 5 times wet weight. The pH of the sodium polyacrylate solution was adjusted with lactic acid so that at the end of the 24-hour treatment the pH was about 4.8. The leather was washed 10 minutes in lukewarm water, drained and cut in half. One-half was fat-liquored in a system conventionally employed with mineral tanned skins and tacked out to dry. The other half was drummed intermittently in a 46.5° Bk. sulfited quebracho solution for 20 hours, rinsed 2 minutes with water, fat-liquored and tacked out to dry. The alum-sodium polyacrylate tannage produced a white, full, well-tanned leather with a shrinkage temperature of 89° C. Retannage of this leather with sulfited quebracho produced a leather that was full, soft, well tanned, even-colored and had a shrinkage temperature of 110° C.

In the preceding examples the range of total  $\text{Al}_2\text{O}_3$  content was from 3.2 to 5.5%; water soluble  $\text{Al}_2\text{O}_3$ , 0.3 to 1.6%; fixed  $\text{Al}_2\text{O}_3$ , 2.9 to 4.4%. For comparison a pickled calfskin control was tanned under the same conditions with a solution of a water soluble basic aluminum acetate at pH of 4.8 but received no further treatment. Analysis of this control piece showed 4.6% total  $\text{Al}_2\text{O}_3$ , 3.0% water soluble  $\text{Al}_2\text{O}_3$ , and 1.6% fixed  $\text{Al}_2\text{O}_3$ . Comparison of the water soluble and fixed  $\text{Al}_2\text{O}_3$  values shows that the polymers of acrylic acid and sodium polyacrylate bind the aluminum salts in the leather, preventing them from being hydrolyzed and washed out.

Vegetable tannin easily and quickly penetrated the "alum-polyacrylate" tanned skin and produced a soft, pliable, fully tanned leather with a uniform color and with a shrinkage temperature well above 100° C. For the vegetable retanned leathers of Examples I and IV the range of total  $\text{Al}_2\text{O}_3$  content was from 2.2 to 3.5%, water soluble  $\text{Al}_2\text{O}_3$ , 0.2 to 0.3%, and fixed  $\text{Al}_2\text{O}_3$ , 2.0 to 3.2%. When a skin tanned only with a water soluble aluminum salt is retanned with vegetable tannin, practically all of the aluminum salt is displaced by the vegetable tannin (0.1 to 0.2%  $\text{Al}_2\text{O}_3$  remains) and forms a sludge or precipitate on both surfaces of the skin, resulting in a very poor leather.

*Example V*

A piece of Iranian sheepskin was drummed in a solution of aluminum sulphate containing 3%  $\text{Al}_2\text{O}_3$  based on the wet drained weight of the skin (403 grams) and 10% (w/v.) sodium chloride. The float ratio was 3 times wet weight skin. The aluminum sulphate

$\text{Al}_2(\text{SO}_4)_3 \cdot 18\text{H}_2\text{O}$  was "masked" with anhydrous sodium acetate; one mole  $\text{Al}_2(\text{SO}_4)_3 \cdot 18\text{H}_2\text{O}$  (79 grams) to one mole of anhydrous sodium acetate (9.7 grams). This solution was basicified with anhydrous sodium carbonate, based on 1/4 of the weight of aluminum sulphate. A pH of 4.10 was obtained after drumming the skin 1 1/2 hours. Sufficient anhydrous sodium carbonate was added in two feeds to bring the final pH to 4.8 after a 24-hour tannage. The skin was removed, washed for 5 minutes in water, drained and drummed in a solution of high molecular weight sodium polyacrylate containing 2% on the wet drained weight skin and 10% (w/v.) sodium chloride for a period of 24 hours. The float ratio was 3 times wet weight. The pH of the sodium polyacrylate solution was adjusted with lactic acid so that the final pH at the end of the tanning period was 4.9. The leather was washed 30 minutes in water and drained. The aluminum sulphate polyacrylate tannage produced a white leather that was full and well tanned with a shrinkage temperature of 80° C. and with a high fixed  $\text{Al}_2\text{O}_3$ .

The aluminum sulphate-polyacrylate tanned skin was fat-liquored with a commercial fat-liquor in the conventional aqueous system. The entire system of fat-liquoring was conducted at 120° F. The fat-liquor was well exhausted after 30 minutes to 1 hour drumming. The product from the fat-liquoring of the skin tanned by the

two step aluminum sulphate-polyacrylate process is a slightly off-white colored leather. The oil penetrated well, making the product flexible and quite soft. Area shrinkage and loss of  $\text{Al}_2\text{O}_3$  during fat-liquor were negligible.

For comparative purposes the following examples are included to demonstrate the results obtained when the sequence of applying the aluminum salt and the polymer are altered.

*Example VI*

A piece of sheepskin was tanned by a process similar to that described in Example IV with the exception that the basic aluminum acetate was equivalent to 3%  $\text{Al}_2\text{O}_3$ , based on wet weight skin. Float ratios were 4 to 1.

A comparable piece of sheepskin was treated with solutions containing exactly the same concentration of reagents but the process was reversed, applying the solution of sodium-polyacrylate first.

Tanning process conditions, such as time skin was in each solution, pH, and temperature were the same in each instance.

The tanned skins were fat-liquored by conventional commercial fat-liquoring processes. Area shrinkage and loss of aluminum salt (determined as  $\text{Al}_2\text{O}_3$ ) was negligible for the skin from the process in which the tanning with aluminum salt was followed by application of the polymer solution. A satisfactory fat-liquored leather was obtained. Attempts to fat-liquor the leather from the process in which the "alum" tannage followed the application of the solution of polymer were unsuccessful, resulting in unsatisfactory leathers.

*Example VII*

A pickled Iran sheepskin was cut along the backbone to give two comparable halves of skin.

One half-skin was tanned with a solution containing water soluble basic aluminum acetate equivalent to 3%  $\text{Al}_2\text{O}_3$  wet weight drained skin, 2% low molecular weight sodium polyacrylate (calculated on same weight skin) and 10% (w/v.) sodium chloride. This solution was adjusted to pH 4.8 with borax solution. The skin was drummed according to standard procedure in this solution containing both aluminum salt and polymer. Float ratio was about 4 to 1 and temperature 85° F. The pH dropped slowly to 4.5 over a period of about 5 hours. The pH was readjusted to 4.8 and drumming continued for a total of 24 hours. The tanned skin was washed, drained and fat-liquored by drumming for one and one-

half hours at 120° F. in a system similar to that used in the trade for mineral tanned skins.

The oil did not penetrate well into this skin, being on the surface, especially on the flesh side. The grain surface was coarse and rough and the leather lacked flexibility. The shrinkage to about two-thirds the area considered normal for this process was excessive. This leather would be rejected in the trade.

The other half of the pickled Iran sheepskin was tanned

10 according to the two-step process of the present invention. The skin was first drummed for 24 hours in a solution containing aluminum salt equivalent to 3%  $\text{Al}_2\text{O}_3$ , based on wet weight drained skin and 10% (w/v.) sodium chloride adjusted to pH 4.8 and at 85° F. The skin was

15 then drummed in a solution containing 2% low molecular weight sodium polyacrylate based on wet weight skin and 10% (w/v.) sodium chloride, pH 4.8, at 85° F. for 24 hours. Float ratios were about 4 to 1.

The tanned skin was washed, drained and fat-liquored

20 substantially as described for the other half-skin. The oil penetrated well, making the leather flexible and quite soft. Shrinkage and loss of aluminum salt during fat-liquoring were negligible.

In addition to those mentioned, the process of this invention may be applied to other types of skins, and to

bated as well as pickled skins.

We claim:

1. A process for tanning skins comprising impregnating the skins with a solution of a water soluble aluminum salt until the skins are tanned, and subjecting the tanned skins to the action of a water soluble material selected from the group consisting of homopolymer of acrylic acid, sodium polyacrylate and ammonium polyacrylate, to fix the aluminum salt in the tanned skins, and subjecting the thus tanned skins to an aqueous fat-liquoring treatment.

2. A process according to claim 1, wherein the aluminum salt is basic aluminum acetate and the water soluble material is sodium polyacrylate.

References Cited in the file of this patent

UNITED STATES PATENTS

2,205,883 Graves ----- June 25, 1940  
2,328,901 Grimm ----- Sept. 7, 1943

FOREIGN PATENTS

530,643 Great Britain ----- Dec. 17, 1940  
552,122 Great Britain ----- Mar. 24, 1943  
569,385 Great Britain ----- May 22, 1945